

## [54] METHOD AND APPARATUS FOR JOINING THE ENDS OF ALUMINUM CONDUCTORS BY CASTWELDING

[75] Inventors: William C. McMurray, St. Clair Shores; Mitchell D. Charneski, Southfield, both of Mich.

[73] Assignee: The Detroit Edison Company, Detroit, Mich.

[22] Filed: Jan. 2, 1973

[21] Appl. No.: 320,105

[52] U.S. Cl. .... 164/333, 164/108, 164/334, 164/337, 164/338, 249/78, 249/79, 249/94, 249/95, 249/97

[51] Int. Cl. .... B22d 37/00

[58] Field of Search .... 164/335, 338, 333, 334, 164/337, 332, 108, DIG. 12, 112, 103, 105, 98, 100, 250; 249/97, 78, 79, 96, 83, 90, 93, 94, 95, 85, 86, 91

## [56] References Cited

## UNITED STATES PATENTS

1,747,419 2/1930 Bottrill..... 249/96 X

|           |         |                   |             |
|-----------|---------|-------------------|-------------|
| 1,838,357 | 12/1931 | Bottrill.....     | 164/DIG. 12 |
| 2,171,778 | 9/1939  | Yantis.....       | 164/335 X   |
| 3,004,310 | 10/1961 | Burke .....       | 249/96      |
| 3,233,292 | 2/1966  | Kramer et al..... | 164/108 X   |

## FOREIGN PATENTS OR APPLICATIONS

948,354 1/1949 France .....

Primary Examiner—Francis S. Husar

Assistant Examiner—V. K. Rising

Attorney, Agent, or Firm—Whittemore, Hulbert &amp; Belknap

## [57] ABSTRACT

The ends of large aluminum conductors are confined in juxtaposition in a preheated mold. in an inert atmosphere molten aluminum is first caused to flow across the exposed ends of the conductors, remove impurities, and is thereafter confined to surround and join the end portions of the conductors at which time it is solidified.

4 Claims, 3 Drawing Figures



PATENTED JAN 14 1975

3,860,062



**METHOD AND APPARATUS FOR JOINING THE  
ENDS OF ALUMINUM CONDUCTORS BY  
CASTWELDING**

**BRIEF SUMMARY OF THE INVENTION**

The present invention relates to a method and apparatus for economically joining the ends of large aluminum conductors by castwelding. The invention is applicable to either clean conductors or conductors which may be covered with oil or which may include multiple strands with oil within the conductor. The invention produces a metallurgical bond of high electrical conductivity and high tensile strength.

The castwelding is accomplished by first melting an electrical grade aluminum in a portable furnace with the aluminum protected from oxidation (argon or another inert gas). Then the molten aluminum is channeled into a preheated mold containing the bared connector ends positioned in juxtaposition to each other. While the mold cavity is under the same protective atmosphere, the molten aluminum is directed against the end faces of the conductors contained therein. Impingement of the melted aluminum cleans the oxide and oils from the conductor ends so that a fusion or metallurgical bond of the aluminum conductors and melted metal is caused to occur. The temperature of the molten aluminum is sufficiently high so that it will produce at least some melting of the surface portions of the aluminum cable, thus causing the impurities and contaminants to flow away from the bared conductor ends.

All heating of the aluminum which constitutes the joint is done outside the weld zone, thus only the minimum heat necessary to melt the required amount of aluminum for the joint, plus a small amount of surplus heat to melt part of the strands, and to compensate for slight losses, is required. The cable therefore requires minimum cooling after the castweld operation.

Cooling clamps are attached to the cable on each side of the mold to limit conduction of heat from the mold and thereby to maintain temperatures within the conductor exterior of the mold below temperatures which would be deleterious to conductor insulation (120° C.).

The mold and cooling clamps may be cooled by controlled circulation of compressed air or CO<sub>2</sub>.

**BRIEF DESCRIPTION OF THE DRAWING**

FIG. 1 is a vertical section through the apparatus.

FIG. 2 is a vertical section taken 90° from the sectional view of FIG. 1.

FIG. 3 is an elevational view of the front of the control console.

**DETAILED DESCRIPTION**

FIGS. 1 and 2 illustrate the apparatus as applied to producing a castweld joint in a four-sector compact strand aluminum conductor having an outside diameter of approximately 1 1/4 inch. It will thus be seen that the apparatus is extremely compact and that for producing a castweld joint on large aluminum cable of this size the overall height of the apparatus is only slightly over 14 inches.

The apparatus thus is quite small and readily portable, and has extremely useful characteristics of a device for making joints in confined spaces such as manholes.

Moreover, as will subsequently be described in detail, the furnace power for melting the aluminum is supplied from electrical resistance heating elements operable on low commercial voltages such for example as 220 volts, thus providing a safety factor where the apparatus is used in damp or wet confined spaces such as manholes.

The aluminum is melted in a portable furnace indicated generally at 10 which comprises a carbon crucible 12 surrounded by high temperature insulation 14 such as aluminum silicate surrounded by a stainless steel jacket 16. Preferably, the stainless steel jacket is surrounded or partly surrounded by a rugged metal screen 18 spaced at a small distance from the steel jacket to provide an air space and to allow the user to handle the pot, should the need arise, even after it has reached maximum temperature.

An opening 20 is provided at the bottom of the crucible 12 and flow of molten aluminum through the opening 20 is controlled by a carbon gate 22 having a port 24 adapted to be moved in registration with the elongated opening 20 by suitable actuating means such for example as a solenoid indicated generally at 26. When energized, the solenoid is adapted to shift the port 24 into registration with the opening 20 and to permit molten aluminum to flow downwardly out of the carbon crucible 12. Suitable means such for example as a spring (not shown) is provided for moving the gate 22 to the closing position illustrated in FIG. 2.

Directly adjacent the outer surface of the carbon crucible 12 are heating means 28 which include electrical resistance heating elements 30.

Means are provided for evacuating air from the furnace and this means is indicated as a conduit 32 for forcing argon or another inert gas into the furnace to evacuate air therefrom.

Means are provided for sensing the temperature of the aluminum in the crucible and this means is shown as a thermocouple 34 embedded in the carbon crucible and having an external connection 36 to suitable automatic control means responsive to temperature of the aluminum in the crucible.

Below the furnace 10 is a mold assembly indicated in its entirety at 40 and comprising a steel mold 42 having a horizontal through opening 44 intersecting a vertical through opening 46. The lower end of the through opening 46 is provided with a closure 48 dividing the vertically extending through opening 46 into a mold well 50, a riser passage 52, and intermediate the mold well and riser passage, the mold cavity 54 which surrounds the ends of the aluminum electrical conductors 56. The horizontally extending opening 44 is slightly larger than the diameter of the conductors 56 and receives collars 58 which limit flow of molten aluminum longitudinally of the cable from the intermediate portion of the mold cavity 54.

In the specific construction illustrated the collars 58 may have a wall thickness of approximately 5/32 inches, and the inner ends thereof may be spaced approximately 1 1/4 inches from the vertical opening 46.

A connection 59 is provided for causing an inert gas such for example as argon to flow into the mold and to displace air from the mold so that the formation of the castweld may take place in an inert atmosphere.

The steel mold 42 is provided with electrical resistance heating elements 60 having external connections indicated at 62 for the purpose of preheating the mold and the ends of the conductor therein to a temperature

slightly below the melting temperature of aluminum. The steel mold 42 is further provided with passages diagrammatically indicated at 64 through which cooling fluid may be circulated following pouring of the molten aluminum. The cooling fluid may be air, CO<sub>2</sub>, or the like.

The steel mold 42 is surrounded by high temperature insulation 66 such for example as aluminum silicate surrounded by a steel jacket 68.

The furnace 10 and the mold assembly 40 are interconnected by flanged tubular portions indicated generally at 70 suitably secured together as for example by screws 72.

It will be appreciated of course that the mold assembly 40 must be formed in two pieces to permit removal of the castweld joint following solidification of the molten metal, and this arrangement is indicated diagrammatically by the partition line 74.

Means 76 provide a local cooling action to the portions of the conductors directly adjacent the exterior of the mold assembly 40. This means comprises a two-piece removable cooling clamp having connections 78 and 80 for circulating a cooling fluid such for example as air, CO<sub>2</sub>, or the like.

The furnace 10 includes a sealing and insulating cover 82 including an insulating core 84 surrounded by a steel shell 86. The cover is adapted to be clamped in closing position at the upper end of the furnace by suitable means such, for example, as screws 88, apertured ears 90, and wing nuts 92.

In use the ends of the electrical conductors 46 are preferably beveled as indicated at 94 and the beveled surfaces are positioned to be exposed upwardly to cause molten aluminum discharged from the crucible 12 to flow across the beveled surfaces. In order to produce the most effective flow of molten aluminum, the lower end of the crucible, below the gate 22, is provided with a pour spout 96 having two nozzles 98 each of which is provided with an elongated passage for directing molten aluminum to one of the beveled surfaces 94. Accordingly, the pour spout divides the flow of molten aluminum into two paths each of which is directed to one of the beveled surfaces of the cable 56.

The steel molds 42 are designed to do five things: First, the electric heating elements in the mold preheat the mold and cable parts prior to the pouring operation. Secondly, the well of the mold permits a substantial flow of molten aluminum across the ends of the aluminum conductor and provides a space for storage of the surplus aluminum together with the contained contaminants below the cable ends to facilitate the making of a castweld joint between clean cable ends. Third, the provision of mold space of slightly larger diameter than that of the cable around the cable ends aids in preheating the conductor and permits the solidified metal to grip the cable strands inwardly from the end and outer surfaces for additional tensile strength. Fourth, passages in the mold provide for flow of coolant in properly timed relation in the cooling cycle to achieve a desirable fine grain (equi-axed) structure. Fifth, risers of proper size plus the preheat and operational procedures eliminate the common defects associated with casting or welding of aluminum. Such defects which have been eliminated by the present method and apparatus are shrink holes, gas pockets, shrink cracks, large grain size, and poor interface weld. Accordingly, there

is a consequent increase in aluminum purity, strength, and conductivity.

The cooling clamps indicated at 76 are designed to feed compressed air or CO<sub>2</sub> gas across and around the cable strands, and are not designed to act as conductive cooling fins. For this reason they may be made of any rugged material capable of withstanding about 300° F. continuously.

The apparatus as described in the foregoing may be operated manually, but in order to insure that an inexperienced splicer may obtain perfect welds each time, it is preferred to automate the operation.

In FIG. 3 there is illustrated a control console 100. Within the console are the valves and switches necessary to perform automatic cycling of the apparatus. As illustrated, the console includes an inlet connection 102 and an outlet connection 104 for inert gas such as argon. An inlet connection 106 is provided for compressed air or CO<sub>2</sub>, and outlet connections 108 and 110 are provided for supplying the cooling fluid to the cooling clamps 76 and the cooling passages 64 of the steel mold 42. Input electrical connection means 112 are provided. An outlet fitting 114 is provided for connection of the heating current to the electrical heating elements 28 and 60. A fitting 116 is provided for connection to the thermocouple.

A main "ON" and "OFF" switch 118 is provided and a selector switch 120 is provided for selecting either manual or automatic control.

For manual control the appropriate switches are provided with manually operable actuators and these switches are indicated at 122, 124, 126, 128 and 130. Associated with each of the switches is a signal light 132 which may be of appropriately different colors. For example, the switch 122 may supply current to the heating elements 28, and if desired, a similar but separate switch (not shown) may be provided for controlling the circuit to the heating element 60 provided in the mold 42. Actuation of the solenoid 26 may be under the control of the switch 124. The switch 126 controls the flow of coolant to the cooling clamps 76, and the switch 128 controls flow of coolant to the cooling passages 64 in the mold. The switch 130 terminates the cycle.

With the switch 120 in the position to select automatic operation, current is supplied to heating elements 28 and the temperature is sensed by the thermocouple 34. When the temperature has risen a predetermined amount, or when a predetermined time interval has passed, the switch supplying current to the mold heating elements 60 is closed. When the aluminum has been completely melted and attained the proper temperature as sensed by the thermocouple, the solenoid 26 is energized actuating the gate valve and permitting the melted aluminum to flow downwardly and be divided by the pour spout into two streams, each of which flows across the exposed end surface of the aluminum cables, carrying away the oxide at the surface and any impurities or contaminants which may be present. These are trapped within the mold well and as the pouring operation continues, the pure molten aluminum rises across the end surface of the conductors and enters the riser passage 52. At this time the switch 126 is operated to direct flow of coolant through the cooling clamps 76 and shortly thereafter, the switch 128 is operated to direct coolant to the passages 64 within the mold 42. The heating elements 28 and 62 are of course

de-energized by operation of the switches controlling the current thereto at the appropriate point in the cycle. As soon as the mold has cooled sufficiently the operation is complete and the cables with the castweld joint are removed from the mold. At this time the lateral projections formed by the solidified material in the mold well and in the riser passage may be mechanically removed.

In the foregoing it has been implied that the quantity of aluminum melted in the pot is that amount which is required for the production of a single weld. The invention however, contemplates the possibility that the pot may be substantially enlarged and the cycle changed to maintain a supply of molten aluminum within the crucible as a plurality of castwelds are made. This requires that the timing of the operation of the carbon gate 22 shall be such as to meter a measured amount of molten aluminum into the mold. With this operation a number of joints may be produced in a shortened time since the time cycle will not require melting of a charge of aluminum for each operation.

There are many advantages in the method and apparatus disclosed herein. In the first place, substantial economies are achieved because of inexpensive equipment. The apparatus is simple and can be operated by inexperienced splicers. The operation is very fast operating including the time cycle required for melting the aluminum and the time cycle for solidification of the cast metal, all of which permits the production of multiple splices.

Since the castweld is produced by high purity electrical grade aluminum melted in an inert atmosphere in an operation which substantially eliminates contaminants from within the weld zone, the joints have high electrical conductors and produce a bond superior to previously known methods. As a consequence, the joints have high tensile strength and allow long pulls of conductors between separated manholes. The joints are corrosion resistant since they are made of electrical grade aluminum as is the conductor.

Since the operation as described, is effective to carry away oil or other contaminants which may be present at and adjacent the ends of the cables, the operation requires no solvents or water.

A very important advantage of the apparatus and method disclosed herein is its low power requirements.

The foregoing advantages become particularly apparent when compared with two prior welding methods which have some times been used. The prior welding methods are: The inert-gas arc welding method, and induction welding. The inert-gas arc welding method suffers from the tedious requirement of cleaning with solvents even the slightest traces of oil from the conductor in order to obtain a useful bond. Tensile strengths are as low as one-third of the breaking strength of the cable. The use of solvents in a manhole of restricted space pose obvious hazards. Furthermore, the arc welding method requires the services of two specially trained welders with costly equipment.

Induction welding as applied to cables of the type disclosed herein, requires about 100 kva of instantaneous power plus a cooling water supply. These are highly undesirable requirements, particularly in carrying out the induction welding in manholes where problems are encountered as a result of the use of extremely heavy and bulky transformer equipment.

The castweld system appears to have significant advantages in every aspect of its application and use. What we claim as our invention is:

1. Apparatus for castweld joining of large aluminum conductors which comprises an insulated pot for melting a charge of aluminum, heating means incorporated into the pot, said pot having a gate-controlled opening at the bottom thereof, a mold directly below the bottom opening in said pot, said mold having a mold cavity for receiving the bared ends of two conductors to be joined by castwelding, a well extending downwardly from said cavity, means for locating the conductor ends in position such that melted aluminum discharged from said pot flows over them and into said well, and a riser passage extending upwardly from said mold cavity, in which said heating means comprises electrical resistance heating elements operable at low commercial voltages to melt aluminum in said pot, said mold cavity being defined by the intersection of a vertical cylindrical opening, the lower portion of which forms said well and the upper portion of which forms said riser passage, and a horizontal cylindrical opening, the portions of which adjacent said vertical opening are slightly larger than the conductors to be joined to provide for a flow of melted aluminum along the outer surface of said conductors, said mold comprising a two-piece metal block having said horizontal and vertical openings therein, the division between the two pieces of said block being in a vertical plane bisecting said horizontal and vertical openings, and mold preheating means comprising low voltage electric heating elements incorporated therein, said mold having mold cooling means comprising flow passages therein for receiving a fluid coolant to accelerate solidification of molten aluminum after pouring the molten aluminum into said mold, and means for circulating the coolant through said flow passages.

2. Apparatus for castweld joining of large aluminum conductors which comprises an insulated pot for melting a charge of aluminum, heating means incorporated into the pot, said pot having a gate-controlled opening at the bottom thereof, a mold directly below the bottom opening in said pot, said mold having a mold cavity for receiving the bared ends of two conductors to be joined by castwelding, a well extending downwardly from said cavity, means for locating the conductor ends in position such that melted aluminum discharged from said pot flows over them and into said well, and a riser passage extending upwardly from said mold cavity, comprising in addition means for dividing the flow of molten aluminum into two parts, and directing each part against the ends of one of the conductors.

3. Apparatus as defined in claim 2 comprising means for supporting the conductor ends in spaced relation.

4. Apparatus for castweld joining of aluminum conductors which comprises a mold having a cavity for receiving the ends of horizontally disposed aluminum conductors in proximity to each other, a well disposed beneath said cavity to receive melted metal flowing downwardly through said cavity over the proximate surfaces of the conductors, said mold having a horizontally extending opening therethrough intersecting said mold cavity, the outer portions of said opening dimensioned to closely embrace portions of conductors received therein, the portions of said opening adjacent said mold cavity being slightly enlarged to provide an annular chambers dimensioned to permit a flow of molten

aluminum into said chambers and to surround portions of said conductors adjacent the ends thereof, a riser passage extending upwardly from said cavity to channel a flow of melted metal into said cavity and to receive excess melted metal after said cavity and well are filled, and means for supplying controlled amounts of melted

metal to said riser passage, said mold cavity having low voltage electrical resistance heating elements incorporated therein and in addition having passages for the circulation of cooling fluids therethrough to control the cooling cycle of melted metal therein.